

Jan. 26, 1954

G. E. MURRAY

2,667,453

METHODS OF ELECTROPLATING COPPER ON METAL ARTICLES

Filed June 3, 1950



FIG. 1



FIG. 2

INVENTOR  
G. E. MURRAY  
BY *G. E. Murray*  
ATTORNEY

## UNITED STATES PATENT OFFICE

2,667,453

METHOD OF ELECTROPLATING COPPER  
ON METAL ARTICLES

Guy E. Murray, Towson, Md., assignor to Western Electric Company, Incorporated, New York, N. Y., a corporation of New York

Application June 3, 1950, Serial No. 165,985

11 Claims. (Cl. 204—28)

1

This invention relates to methods of electroplating copper on metal articles, and more particularly to methods of electroplating conductive layers of copper on steel wires.

In the manufacture of composite conductors including a steel core and a conductive copper covering enclosing the steel core, it has been proposed in the past to form the copper covering by electrodeposition upon the steel core. However, in the prior art methods it has been impossible to produce economically a composite conductor including steel wire having a thick, fine-grained, nonporous, copper covering, because whenever the current densities used on the core were sufficiently high to make the electroplating process economically feasible, the resulting coverings were coarse-grained and generally unsatisfactory.

An object of the invention is to provide new and improved methods of electroplating copper on metal articles.

A further object of the invention is to provide new and improved methods of electroplating copper on steel wires.

Another object of the invention is to provide new and improved methods of electroplating tenaciously adherent, fine-grained, nonporous, thick copper coverings on steel cores at high rates of speed.

An additional object of the invention is to provide new and improved methods of electroplating heavy, electroconductive layers of copper on high strength steel wires to produce composite conductors suitable for use in communication systems, and the like.

A method illustrating certain features of the invention may include electroplating a very thin, fine-grained, copper flash deposit on a metal article in an alkaline bath having a predetermined low copper concentration therein, electroplating a heavier, protective deposit of copper on the fine-grained deposit in a second alkaline bath having a concentration of copper therein substantially greater than that in the first-mentioned bath, and then electroplating a heavy deposit of copper on the article in an acid copper plating bath.

A complete understanding of the invention may be obtained from the following detailed description of a method forming a specific embodiment thereof, when read in conjunction with the appended drawing, in which:

Fig. 1 is a schematic view of an apparatus for practicing a method forming one embodiment of the invention, and

Fig. 2 is a longitudinal, vertical section of a copper plating cell forming a portion of the apparatus shown in Fig. 1.

2

A wire 10 composed of high tensile strength, high carbon steel is withdrawn from a supply 11 thereof by a capstan 12. In order to prepare the wire for electroplating copper thereon, it is advanced continuously by the capstan 12 through a degreaser 14, which applies trichloroethylene or other suitable degreasing solvent, to the wire to remove grease therefrom. The wire then passes successively through an alkaline electrolytic cleaning cell 15, which cleans the surface of the wire, a water rinsing bath 16, which washes the alkali material from the surface of the wire, an acid electrolytic cell 17, which preferably contains sulphuric acid and further cleans the surface of the wire 10, and a water rinsing bath 18, which rinses the acid from the wire.

The cell 15 preferably contains an electrolyte consisting of a water solution of sodium orthosilicate having a concentration of from about 3.0 to about 7.0 ounces per gallon of water. The electrolyte in the cell 15 is kept at a temperature within the range of from about 140° F. to about 200° F. Positive contact sheaves 19—19 which engage the wire 10 and a suitable cathode 20 cause an electric current to flow through the wire and the electrolyte in the cell 15. The current density on the wire in the cell 15 is maintained at a value within the range of from about 50 to about 200 amperes per square foot.

The cell 17 preferably contains an electrolyte composed of a sulphuric acid solution having a concentration of from about 5% to about 25%, and the electrolyte is maintained at a temperature below 110° F. Positive contact sheaves 21—21 in engagement with the wire 10 and a cathode 22 cause an electric current to flow through the wire and the electrolyte at a current density on the wire from about 400 to about 1000 amperes per square foot.

The degreaser 14, the cells 15 and 17 and the baths 16 and 18 clean the surface of the wire 10 thoroughly so that the wire is very smooth and clean. The wire then is advanced as a cathode through a flash plating cell 24 having a low copper concentration, alkaline cyanide electrolyte to apply a very fine-grained, thin flash deposit on the wire. This thin copper deposit is applied at a cathode current density which, generally speaking, is low but which is a high current density for the copper concentration of the electrolyte. The grain structure of the flash deposit thus applied sets the pattern for subsequent deposits of copper substantially independently of copper concentration of the baths and current densities employed in applying those deposits. This flash deposit of copper adheres tenaciously to the wire. The wire then is advanced as a cathode through

a plating cell 26 having a high copper concentration, alkaline cyanide plating bath to apply a further deposition of fine-grained copper on the flash deposit. A high cathode current density is maintained in the cell 26 to produce a high rate of copper deposition to build up the copper deposit rapidly to a thickness sufficient for plating thereon in subsequent acid plating baths without galvanic deposition of copper thereon. The wire is advanced continuously from the cell 26 through a water rinsing bath 28, and an acid bath 29 to wash off and neutralize any alkali on the wire. The wire then is advanced continuously as a cathode through acid plating cells 31, 32, 33 and 34, which plate copper on the previous deposit with very high current densities on the wire and very high rates of deposition.

The plating cell 24 may be constructed somewhat like that shown in Fig. 2, and consists of a conductive anode compartment 36 having slots 37-37 in the end walls thereof through which the wire 10 passes. A layer 38 of finely divided copper, such as scrap copper or small copper balls, rests on the bottom of the anode compartment 36, and the electrolyte employed is fed into the bottom of the compartment by means of inlet pipes 39-39. The electrolyte flows from the inlet pipes 39-39 through the layer 38 of finely divided copper, and out of the compartment 36 through the slots 37-37. The overflow falls into an outer compartment 40 from which it flows into a suitable tank (not shown), which serves as a reservoir from which the electrolyte is pumped through the inlet pipes 39-39.

The anode compartment 36 is connected to the positive side of a source of D. C. potential, thereby by making the layer 38 of finely divided copper the anode in the cell 24, and the anode compartment is insulated from the outer compartment 40. The finely divided copper dissolves anodically to replenish the electrolyte with copper ions as copper is plated on the wire 10. Finely divided copper is added to the layer 38 from time to time to maintain an adequate supply of anode material. Contact sheaves 42-42, which are connected to the negative side of the D. C. source, are engaged by the wire 10, whereby the wire is made the cathode in the plating cell 24.

The copper concentration of the electrolyte in the cell 24 is low so that a very thin, fine-grained, flash deposit of copper is applied to the wire 10. This flash deposit is pure and very fine-grained in structure due to the diluteness of copper in the electrolyte in this cell, and it is tenaciously adherent to the wire because of the purity, denseness and fine-grained structure of the deposit. The cathode current density, which is kept sufficiently low for the low concentration of copper in the cell 24, should not be greater than about 75 amperes per square foot, and preferably should be between about 20 and about 50 amperes per square foot. The temperature of the bath is maintained at from about 140° F. to about 180° F.

A highly satisfactory electrolyte for use in the cell 24 is a mixed copper-potassium cyanide electrolyte having a composition within approximately the following limits:

|                            | Oz. per gal. |
|----------------------------|--------------|
| Copper (as cyanide)        | 1.5 to 3.0   |
| Potassium cyanide (free)   | 0.1 to 1.0   |
| Potassium hydroxide (free) | 3.0 to 6.0   |
| Potassium carbonate        | 6.0 to 7.5   |

The most important elements of this type of electrolyte are the copper content and the free

potassium cyanide content thereof. The preferred limits for the copper content are from 1.75 to 2.5 ounces per gallon, while the preferred limits for the free potassium cyanide content are from 0.3 to 0.7 ounce per gallon.

Negative contact sheaves 46-46 are provided adjacent to the cell 26 which is similar to the cell 24 and includes an anode 48 composed of divided metallic copper. A heavy deposit of copper is applied to the wire 10 in the cell 26 to protect the wire against galvanic cell copper deposition thereon in the acid plating cells 31, 32, 33 and 34. A deposit of from about 0.0001 inch to about 0.0002 inch is applied in the cell 26 under a substantially higher current density than was used in the cell 24. The deposit applied to the wire in the cell 26 is very fine-grained and dense inasmuch as the flash deposited on the wire in the cell 24 had already set the crystalline pattern of further deposits of copper.

A very satisfactory electrolyte for use in the cell 26 is a mixed copper-potassium cyanide bath having a composition within about the following limits:

|                            | Oz. per gal. |
|----------------------------|--------------|
| Copper (as cyanide)        | 4.5 to 7.0   |
| Potassium cyanide (free)   | 0.0 to 1.0   |
| Potassium hydroxide (free) | 3.0 to 6.0   |
| Potassium carbonate        | 6.0 to 7.5   |

Here again, the concentrations of the copper and of the free cyanide are the most important elements of the electrolyte. The copper concentration preferably is within the range of from 4.5 to 6.5 ounces per gallon, and the free cyanide content preferably should be from 0.3 to 0.7 ounce per gallon.

The difference of potential between the contact sheaves 46-46 and the anode 48, the spacing of the anode from the path of the wire and the electrical resistance of the electrolyte are such that a cathode current density of from about 50 to about 200 amperes per square foot is maintained in the cell 26, the current density being kept substantially higher than that in the cell 24. The cell 26 is kept at a temperature of from about 140° to about 180° F.

The wire 10 emerges from the cell 26 having a plated copper covering thereon which is sufficiently thick to protect it against galvanic deposition of copper thereon. The water rinsing bath 28 and the acid bath 29 wash off or neutralize any alkali carried by the wire from the cells 24 and 26. The acid bath 29 may be a hydrofluoboric acid solution at a concentration of from about 1.0 to about 10.0 ounces per gallon, or a sulphuric acid solution at a concentration of from about 1.0 to about 10.0 ounces per gallon, depending on the type of electrolyte employed in the cells 31, 32, 33 and 34. The bath 29 is held at a temperature between about 60° F. and about 100° F. Since electrolyte used in the acid plating cells 31, 32, 33 and 34 may be a copper fluoborate or a copper sulphate solution, if copper fluoborate is used as the electrolyte in these cells, the hydrofluoboric acid solution is used in the neutralizing bath 29, while if copper sulphate is used in these cells, the sulphuric acid solution is used in the bath 29.

The wire 10 is advanced continuously through the cells 31, 32, 33 and 34 at a rate of speed between about 20 feet per minute and about 100 feet per minute, and the electrolytes in the cells are recirculated with a high degree of turbulence. Hence, high current densities may be employed

successfully in plating copper on the conductor without the deleterious action of hydrogen plating. The plating cells 31, 32, 33 and 34 are substantially like the cell 24 in construction, and have finely divided metallic copper anodes. The copper anodes dissolve electrolytically as the plating progresses to maintain the desired copper concentration therein. The wire in passing through the acid plating cells engages contactor sheaves 49-49.

A suitable copper fluoborate electrolyte for the acid plating cells will have a composition within substantially the following limits:

|                            | Oz. per gal. |
|----------------------------|--------------|
| Copper (as fluoborate)     | 7.2 to 20.0  |
| Hydrofluoboric acid (free) | 2.5 to 3.6   |

The electrolyte preferably is operated at a temperature of from about 115° F. to about 136° F., and a cathode current density of from about 500 to about 3000 amperes per square foot is preferred. A good concentration range for these constituents is from about 15 to about 20 ounces per gallon of copper as fluoborate, and from about 3.5 to about 6.5 ounces per gallon of free hydrofluoboric acid. Good results are obtained when a cathode current density of from about 1000 to about 2500 amperes per square foot is employed.

A satisfactory sulphuric acid electrolyte for the acid plating cells will have a composition substantially as follows:

|                       | Oz. per gal. |
|-----------------------|--------------|
| Copper (as sulphate)  | 7.0 to 11.0  |
| Sulphuric acid (free) | 3.0 to 6.0   |

The electrolyte preferably is kept at a temperature of from about 60° F. to about 85° F., and the acid plating cells using this type of electrolyte preferably are operated at a cathode current density of from about 500 to about 1200 amperes per square foot. Excellent results are obtained when the copper concentration is from about 8 to about 10 ounces per gallon, the free sulphuric acid concentration is from about 4.5 to about 5.5 ounces per gallon, and the cathode current density is from about 750 to about 1000 amperes per square foot.

The thickness of copper deposited in the cells 31, 32, 33 and 34 in one particular example has been from about 0.003 inch to about 0.004 inch. The deposit on the wire from the acid plating cells was very fine-grained and dense, being governed by the initial pattern of the grain of the copper deposit in the cyanide cell 24, even though a cathode current density as high as about 3000 amperes per square foot was used.

The covered wire 10 is advanced from the cell 34 to a dragout recovery bath 50 having water therein, and then through a rinsing bath 52. The water in the bath 50 washes any acid on the wire from the cell 34, and forms a dilute acid solution. This dilute acid solution is used to replace the water that is lost from the acid cells 31, 32, 33 and 34 from evaporation and other causes, and water is supplied to replenish it, from the bath 52, if desired.

#### Example I

In electroplating a high carbon, high tensile strength, steel wire having a diameter of 0.032 inch in one successful utilization of the invention, the wire was advanced continuously through the baths and cells 14, 15, 16, 17, 18, 24, 26, 28, 29, 31, 32, 33, 34, 50 and 52 at a rate of speed of 80

feet per minute. Trichloroethylene was used in the degreaser 14, and removed substantially all fats and grease from the wire. Any remaining grease and any other contaminants on the surface of the wire were removed by a sodium orthosilicate solution at a concentration of about 5.0 ounces per gal. in the cell 15, in which the wire was immersed as an anode for 18 seconds at an anode current density of 125 amperes per square foot.

10 The wire was immersed in the acid cleaning cell 17 for 13 seconds as an anode at a current density of 550 amperes per square foot. The electrolyte in the cell 17 was a 15% sulphuric acid solution and was maintained at a temperature of 80° F. The cell 17 cleaned oxides completely from the surface of the wire, so that it was in excellent condition for the electrodeposition of copper thereon.

15 Each portion of the wire was immersed in the flash plating cell 24 for a period of 10 seconds at a cathode current density of 50 amperes per square foot, the period of time being just sufficient to form a thin film or flash thereon. The electrolyte was maintained at a temperature of 150° F. An alkali cyanide electrolyte having the following composition was used as the electrolyte in the cell 24:

|                            | Oz. per gal. |
|----------------------------|--------------|
| Copper (as cyanide)        | 2.1          |
| Potassium cyanide (free)   | 0.5          |
| Potassium hydroxide (free) | 5.0          |
| Potassium carbonate        | 6.0          |

20 The flash deposit of copper produced on the wire in the cell 24 covered the wire completely, and was a thin, strongly adherent, flash film, which was very fine-grained in texture. This film was too thin to measure accurately.

25 Each portion of the wire advanced through the cell 26 was immersed therein for a period of 40 seconds at a cathode current density of 100 amperes per square foot. The cell was kept at a temperature of 150° F. A smooth, dense, very fine-grained deposit 0.00015 inch in thickness was formed on the flash deposit. The electrolyte in the cell 26 had the following composition:

|                            | Oz. per gal. |
|----------------------------|--------------|
| Copper (as cyanide)        | 5.5          |
| Potassium cyanide (free)   | 0.6          |
| Potassium hydroxide (free) | 5.0          |
| Potassium carbonate        | 6.0          |

30 The acid neutralizing bath 29 was a 4% hydrofluoboric acid solution, and was maintained at room temperature (about 70° F.).

35 Each portion of the wire advanced through the acid plating cells 31, 32, 33 and 34 was immersed therein for a total period of 115 seconds at a cathode current density of 1800 amperes per square foot. The electrolytes in these cells were held at a temperature of 128° F. A smooth, dense, fine-grained deposit 0.003 inch in thickness was formed on the wire. The electrolyte in the cells 31, 32, 33 and 34 had the following composition:

|                            | Oz. per gal. |
|----------------------------|--------------|
| Copper (as fluoborate)     | 18           |
| Hydrofluoboric acid (free) | 5.3          |

40 The entire deposit of copper on the wire was uniform, nonporous, dense, tenaciously adherent and fine-grained. There was no "treeing," and the periphery of the deposit was smooth. The temper of the steel wire core was substantially unaffected by the electroplating operation.

7  
*Example II*

A high carbon, high tensile strength, steel wire having a diameter of 0.032 inch was advanced continuously through the baths and cells 14, 15, 16, 17, 18, 24, 26, 28, 29, 31, 32, 33, 34, 50 and 52 at a rate of speed of 80 feet per minute. Trichloroethylene in the degreaser 14 removed substantially all fats and greases from the wire, and this cleaning was completed in the cell 15, having therein an aqueous solution of sodium orthosilicate at a concentration of about 5.0 ounces per gallon in which the wire was immersed for 18 seconds as an anode at a current density of 125 amperes per square foot. The wire was immersed in the cell 17 for 13 seconds as an anode at a current density of 550 amperes per square foot. The electrolyte in the cell 17 was a 15% solution of sulphuric acid, and was kept at a temperature of 180° F. The cell 17 cleaned oxides from the surface of the wire and polished the surface of the wire to a matte condition.

Immersion time of the wire as a cathode in the flash plating cell 24 was 10 seconds, and a cathode current density of 50 amperes per square foot was employed. This immersion time was just sufficient to form a flash film at the current density employed. The temperature of the electrolyte was 150° F. An alkali cyanide electrolyte having the following composition was used in the cell 24:

|                            | Oz. per gal. |
|----------------------------|--------------|
| Copper (as cyanide)        | 2.1          |
| Potassium cyanide (free)   | 0.5          |
| Potassium hydroxide (free) | 5.0          |
| Potassium carbonate        | 6.0          |

The flash deposit of copper applied to the wire in the cell 24 covered the periphery of the wire completely, and was a thin, strongly adherent, very fine-grained film.

Each portion of the wire advanced through the cell 26 was immersed therein as a cathode for a period of 40 seconds at a cathode current density of 100 amperes per square foot. The electrolyte was maintained at a temperature of 150° F. A smooth, dense, very fine-grained deposit 0.00015 inch in thickness was formed on the flash deposit. The electrolyte in the cell 26 had the following composition:

|                            | Oz. per gal. |
|----------------------------|--------------|
| Copper (as cyanide)        | 5.5          |
| Potassium hydroxide (free) | 5.0          |
| Potassium carbonate        | 6.0          |
| Potassium cyanide          | 0.6          |

The acid neutralizing bath 29 consisted of a 10% sulphuric acid solution, and was maintained at a temperature of about 70° F.

Each portion of the wire advanced as a cathode through the acid plating cells 31, 32, 33 and 34 was immersed in these cells for a total period of 230 seconds at a cathode current density of 900 amperes per square foot and at a bath temperature of 70° F. A smooth, uniform, dense, fine-grained deposit 0.003 inch in thickness was formed on the wire. The electrolyte in the cells 31, 32, 33 and 34 had the following composition:

|                       | Oz. per gal. |
|-----------------------|--------------|
| Copper (as sulphate)  | 9.0          |
| Sulphuric acid (free) | 5.0          |

The entire deposit of copper on the wire was uniform, dense tenaciously adherent and fine-grained. The periphery of the deposit was smooth and free of nodes and other projections.

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
80

that causes subsequent deposits on the wire to be similarly fine-grained, maintaining in the second cyanide bath a cathode current density substantially higher than the current density in the flash coating bath to deposit a fine-grained copper coating substantially thicker than the flash coating of copper, and maintaining in the acid plating bath a still higher cathode current density to form a thick copper deposit which increases materially the electrical conductivity of the resulting composite wire.

2. The method of electroplating copper on steel wires, which comprises continuously advancing a steel wire as a cathode seriatim through an alkaline cyanide flash coating bath containing copper dissolved therein at a concentration within the range of from about 1.5 to about 3.0 ounces per gallon, a second alkaline cyanide bath containing a higher concentration of copper dissolved therein, and an acid plating bath containing a still higher concentration of copper dissolved therein, maintaining in the cyanide flash bath a cathode current density within the range of from about 20 to about 75 amperes per square foot for a period of time sufficient to deposit a very thin and very fine-grained flash coating of copper which sets a size pattern that causes subsequent deposits on the wire to be similarly fine-grained, maintaining in the second cyanide bath a cathode current density within the range of from about 50 to about 200 amperes per square foot to deposit a fine-grained copper coating substantially thicker than the flash coating of copper, and maintaining in the acid plating bath a still higher cathode current density to form a thick copper deposit which increases materially the electrical conductivity of the resulting composite wire.

3. The method of electroplating copper on steel wires, which comprises continuously advancing a steel wire as a cathode seriatim through an alkaline cyanide flash coating bath containing copper dissolved therein at a concentration within the range of from about 1.5 to about 3.0 ounces per gallon, a second alkaline cyanide bath containing a higher concentration of copper dissolved therein, and a series of acid plating baths containing a higher concentration of dissolved copper than the concentration in the second alkaline cyanide bath, maintaining in the cyanide flash bath a cathode current density within the range of from about 20 to about 75 amperes per square foot for a period of time sufficient to deposit a very thin and very fine-grained flash coating of copper which sets a size pattern that causes subsequent deposits on the wire to be similarly fine-grained, maintaining in the second cyanide bath a cathode current density within the range of from about 50 to about 200 amperes per square foot to deposit a fine-grained copper coating substantially thicker than the flash coating of copper, and maintaining in the acid plating baths a cathode current density within the range of from about 500 to about 3000 amperes per square foot to form a series of increments of a thick copper deposit which increases materially the electrical conductivity of the resulting composite wire.

4. The method of electroplating copper on steel wires, which comprises advancing continuously a steel wire as a cathode seriatim through an alkaline cyanide, grain-pattern-setting bath having copper dissolved therein at a concentration within the range of from about 1.5 to about 3.0 ounces per gallon, an alkaline cyanide plat-

ing bath having copper dissolved therein at a concentration from about 4.5 to about 7.0 ounces per gallon and an acid plating bath having copper dissolved therein at a high concentration, 5 maintaining a current density on the portion of the wire in the grain-pattern-setting bath within the range of from about 20 to about 75 amperes per square foot and for such a period of time as to just form a very thin, fine-grained, 10 copper, flash deposit on the wire, maintaining a current density on the portion of the wire in the cyanide plating bath within the range of from about 50 to about 200 amperes per square foot to form a fine-grained copper deposit on the flash deposit to protect the wire against galvanic 15 action in the acid plating bath, and electroplating a heavy deposit of copper on the second-mentioned deposit in the acid plating bath at a high cathode current density.

5. The method of electroplating copper on steel wires, which comprises advancing continuously a steel wire as a cathode seriatim through an alkaline cyanide, grain-pattern-setting bath having copper dissolved therein at a concentration of about 2.1 ounces per gallon, an alkaline cyanide plating bath having copper dissolved therein at a concentration of about 5.5 ounces per gallon and an acid plating bath having copper dissolved therein at a very high concentration, 20 causing an electric current of such magnitude to flow through the grain-pattern-setting bath that the current density on the portion of the wire in that bath is from about 20 to about 75 amperes per square foot whereby a very thin, fine-grained, 25 copper flash deposit is formed on the wire, causing an electric current of such magnitude to flow through the cyanide plating bath that the current density on the portion of the wire in that bath is from about 50 to about 200 amperes per 30 square foot to form a fine-grained copper deposit on the flash deposit, and electroplating a heavy deposit of copper on the second-mentioned deposit in the acid plating bath at a very high cathode current density.

6. The method of electroplating copper on steel wires, which comprises advancing continuously a steel wire as a cathode seriatim through an alkali cyanide grain-pattern-setting bath having copper dissolved therein at a concentration from about 1.5 to about 3.0 ounces per gallon, through an alkali cyanide plating bath having copper dissolved therein at a concentration of from about 4.5 to about 7.0 ounces per gallon and through an acid plating bath having copper dissolved therein as copper fluoborate at a copper concentration of from about 7.2 to about 20.0 ounces per gallon, causing to flow through the grain-pattern-setting bath an electric current of such magnitude that the current density on the portion of the wire in that bath is from about 20 to about 75 amperes per square foot and for such a period as to form a very thin, fine-grained, 45 copper, flash deposit on the wire, causing to flow through the cyanide plating bath an electric current of such magnitude that the current density on the portion of the wire in that bath is from about 50 to about 200 amperes per square foot to form a protective, fine-grained, 50 copper deposit on the flash deposit, and electroplating a heavy deposit of copper on the second-mentioned deposit in the acid plating bath at a cathode current density of from about 500 to about 3000 amperes per square foot.

7. The method of forming an electroconductive layer of copper on steel wires, which com-

prises advancing a steel wire continuously as a cathode through a cyanide flash bath containing from about 1.75 to about 2.5 ounces per gallon of copper as cyanide and from about 0.3 to 0.7 ounce per gallon of free potassium cyanide, through a cyanide plating bath containing from about 4.5 to 6.5 ounces per gallon of copper as cyanide and from about 0.3 to 0.7 ounce per gallon of free potassium cyanide, and then through an acid plating bath containing from about 15 to 20 ounces per gallon of copper as fluoborate and from about 3.5 to about 6.5 ounces per gallon of free hydrofluoboric acid, electroplating each increment of the wire passing through the cyanide flash bath at a cathode current density of from about 20 to about 75 amperes per square foot for a period sufficient to form only a thin, fine-grained, flash deposit on the wire, electroplating each increment of the wire passing through the cyanide plating bath at a cathode current density of from about 50 to about 200 amperes per square foot for a period sufficient to form a fine-grained, protective deposit of copper on the flash deposit, and electroplating each increment of the wire passing through the acid plating bath at a cathode current density of at least 500 amperes per square foot for a period sufficient to form a deposit of copper on the protective deposit sufficiently thick to materially increase the electrical conductivity of the resulting composite wire.

8. The method of electroplating copper on steel wires, which comprises advancing continuously a steel wire as a cathode seriatim through a cyanide grain-pattern-setting bath having copper dissolved therein as cyanide at a concentration of 2.1 ounces of copper per gallon, free potassium cyanide at a concentration of 0.5 ounce per gallon, free potassium hydroxide at a concentration of 5.0 ounces per gallon and potassium carbonate at a concentration of 6.0 ounces per gallon, through a cyanide plating bath having copper dissolved therein as cyanide at a copper concentration of 5.5 ounces per gallon, free potassium cyanide at a concentration of 0.6 ounce per gallon, free potassium hydroxide at a concentration of 5.0 ounces per gallon and potassium carbonate at a concentration of 6.0 ounces per gallon, and through an acid plating bath having copper dissolved therein as copper fluoborate at a copper concentration of 18 ounces of copper per gallon, and free hydrofluoboric acid at a concentration of about 5.3 ounces per gallon, electroplating each portion of the wire in the grain-pattern-setting bath for about 10 seconds at a current density of about 50 amperes per square foot whereby a very thin, fine-grained, copper flash deposit is formed on the wire, electroplating each portion of the wire in the cyanide plating bath for about 40 seconds at a current density of about 100 amperes per square foot to form a fine-grained copper deposit on the flash deposit, and electroplating each portion of the wire in the acid plating bath for about 115 seconds at a current density of about 1800 amperes per square foot to form a heavy deposit of copper on the second-mentioned deposit.

9. The method of electroplating copper on steel wires, which comprises advancing continuously a steel wire as a cathode seriatim through an alkaline cyanide grain-pattern-setting bath having copper dissolved therein at a concentration of from about 1.5 to about 3.0 ounces per gallon, through an alkaline cyanide plating bath having copper dissolved therein at a concentration of

from about 4.5 to about 7.0 ounces per gallon and through a sulphuric acid plating bath having copper dissolved therein at a concentration of from about 7.0 to about 11.0 ounces per gallon, maintaining a low current density on the portion of the wire in the grain-pattern-setting bath for such a period of time as to form on the wire a very thin, fine-grained, copper, flash deposit, maintaining a higher current density on the portion of the wire in the cyanide plating bath for such a period of time as to form on the wire a fine-grained copper deposit on the flash deposit to protect the wire against galvanic deposition in the acid plating bath, and electroplating a heavy deposit of copper on the second-mentioned deposit in the sulphuric acid plating bath at a cathode current density of from about 500 to about 1000 amperes per square foot.

10. The method of electroplating a conductive layer of copper on steel wires, which comprises advancing a steel wire continuously as a cathode through a cyanide flash bath containing from about 1.75 to about 2.5 ounces per gallon of copper as cyanide and from about 0.3 to 0.7 ounce per gallon of free potassium cyanide, through a cyanide plating bath containing from about 4.5 to 6.5 ounces per gallon of copper as cyanide and from about 0.3 to 0.7 ounce per gallon of free potassium cyanide, and then through an acid plating bath containing from about 8 to about 10 ounces per gallon of copper as sulphate and from about 4.5 to about 5.5 ounces per gallon of free sulphuric acid, electroplating each increment of the wire passing through the cyanide bath at a cathode current density of from about 20 to about 75 amperes per square foot for a period sufficient to form only a thin, fine-grained, flash deposit on the wire, electroplating each increment of the wire passing through the cyanide plating bath at a cathode current density of from about 50 to about 200 amperes per square foot for a period sufficient to form a fine-grained, protective deposit of copper on the flash deposit, and electroplating each increment of the wire passing through the acid plating bath at a cathode current density of at least 500 amperes per square foot for a period sufficient to form a deposit of copper on the protective deposit sufficiently thick to materially increase the electrical conductivity of the resulting composite wire.

11. The method of electroplating copper on steel wires, which comprises advancing continuously a steel wire as a cathode seriatim through a cyanide grain-pattern-setting bath having copper dissolved therein as cyanide at a copper concentration of 2.1 ounces per gallon, free potassium cyanide at a concentration of 0.5 ounce per gallon, free potassium hydroxide at a concentration of 5.0 ounces per gallon and potassium carbonate at a concentration of 6.0 ounces per gallon, through a cyanide plating bath having copper dissolved therein as cyanide at a copper concentration of about 5.5 ounces per gallon, free potassium cyanide at a concentration of 0.6 ounce per gallon, free potassium hydroxide at a concentration of 5.0 ounces per gallon and potassium carbonate at a concentration of 6.0 ounces per gallon, and through a sulphuric acid plating bath having copper dissolved therein as copper sulphate at a copper concentration of 9.0 ounces per gallon and free sulphuric acid at a concentration of 5.0 ounces per gallon, maintaining in the grain-pattern-setting bath a cathode current density of 50 amperes per square foot for a

period of 10 seconds to form on the wire a very thin, fine-grained, copper, flash deposit, maintaining in the cyanide plating bath a cathode current density of 100 amperes per square foot for a period of 40 seconds to form on the wire a fine-grained copper deposit on the flash deposit to protect the wire against galvanic deposition in the acid plating bath, and maintaining in the acid plating bath a cathode current density of 900 amperes per square foot for a period of 230 seconds to form a heavy deposit of copper on the second-mentioned deposit.

GUY E. MURRAY.

References Cited in the file of this patent

UNITED STATES PATENTS

| Number      | Name               | Date          |
|-------------|--------------------|---------------|
| 5 2,317,350 | Adler et al. ----- | Apr. 27, 1943 |
| 2,420,291   | Adler -----        | May 13, 1947  |

OTHER REFERENCES

Transactions Electrochemical Society, "Modern Electroplating" (special volume), 1942, pp. 155-158, 173-175, 177-178, 186-187.

Transactions Electrochemical Society, vol. 83, 1946, pp. 263-266.